# EUROPEAN PATENT SPECIFICATION

(11) **EP 0 045 662 B1**
(45) Date of publication and mention of the grant of the patent: **28.03.1984**
(21) Application number: 81303576.3
(22) Date of filing: 05.08.1981
(51) Int. Cl.: C10C 3/02

(54) **Modified bitumens and production thereof**
Modifiziertes Bitumen und seine Herstellung
Bitume modifié et sa production

(30) Priority: 05.08.1980 GB 8025512
(43) Date of publication of application: 10.02.1982
(73) Proprietor: EXXON RESEARCH AND ENGINEERING COMPANY, Florham Park, New Jersey 07932-0390 (US)
(72) Inventor: Muller, Jean-Marie Alfred Francois, F-76420 Bihorel (FR); De La Taille, Bruno Marie, F-76000 Rouen (FR)
(74) Representative: Pitkin, Robert Wilfred

## Description

This invention relates to modified bitumens and to a process for producing them. The invention is more especially concerned with bitumens modified chemically, which chemically modified bitumens have improved rheological properties rendering them useful, for example, in roadmaking.

In the past, rheological or other properties of bitumens have been altered in several ways. Thus, for example bitumen has been chemically modified by oxidation (or dehydrogenation), or by treatment with sulphur. For example, chlorides of (i) tin and other metals, (ii) silicon and (iii) phosphorus have been suggested for treating a tar (GB-A-285,000). Chlorides of zinc and other metals and of phosphorus have been mentioned for treating bitumen (GB-A-382842). Metal chlorides, sulphuric acid and phosphoric acid have been disclosed for treating bitumen (GB-A-1,331,609). Further, it has been proposed to catalyse the air/oxygen blowing of bitumen, to give an oxidised bitumen, by means of a catalytic quantity of an anhydrous solution of phosphorus pentoxide in phosphoric acid (GB-A-916,531). The use of phosphorus pentoxide alone as a catalyst in bitumen blowing processes is described in Industrial and Engineering Chemistry Vol. 45 No. 10, Page 2121 ff.

US-A-2673815 discloses the heating of bitumen with phosphorus sesquisulphide, preferably as a dispersion of that compound in an oil miscible with the bitumen. US-A-2676910 discloses the heating of bitumen with phosphorus pentoxide as a reactant rather than as an oxidant catalyst.

Bitumen has also been modified by blending with other materials, for example, synthetic rubbers, natural rubber, various synthetic homo-or co-polymers, and elastomers.

The modified bitumen products have different properties according to the nature of the modification achieved and the manufacturing method employed; the manufacturing methods often being expensive in materials and/or treatment times involved.

There is required at the present time a moderately-priced bituminous binder which has improved fatigue resistance properties and which imparts improved resistance to permanent deformation to surfacings incorporating that binder.

It is one object of the present invention to provide a modified bitumen which, among other characteristics, at least substantially meets the aforesaid requirement for a bituminous binder.

According to the present invention there is provided a chemically modified bitumen possessing phosphorus-containing groups, characterised in that said groups are in the form of a phosphorus-containing compound of a metal, preferably of a polyvalent metal, or of an ammonium group or amine.

The phosphorus-containing groups may be, for example, acidic groups neutralised to form a metal, ammonium or amine salt. They may also be, for example, groups forming an ion with which a metal counter-ion is associated to form a relatively stable product.

Preferably the said phosphorus-containing groups are phosphonic or thiophosphonic groups. The preferred metals are calcium, barium and zinc. Other polyvalent metals which may be employed include magnesium, aluminium and iron. Monovalent metals may be found suitable, for example, potassium and sodium.

In a further aspect, the invention provides a process for the production of a chemically modified bitumen comprising reacting the bitumen with a phosphorus-containing compound, characterised by further reacting the phosphorus-containing groups in the product, directly or after a hydrolysis step, with a metal compound or an amine or an ammonium compound.

For the formation of thiophosphonic groups the preferred compound employed is phosphorus pentasulphide. For phosphonic groups the preferred compound is phosphorus pentoxide. The phosphorus compound is normally employed in a quantity of 0.5 to 25 wt.%, more usually 2 to 7.5 wt.%, preferably 2.5 to 5 wt.%, calculated as phosphorus and based on the wt. of the bitumen. In all cases reaction temperatures are normally in the range 100° to 175°, more usually 125°C to 160°C, preferably 140°C to 150°C. Reaction times depend, at least to some extent, on the final properties required. For example, starting with a bitumen having a softening point ("Ring and Ball" ASTN-D36) of 40°C then an increase to a higher softening point, say 100°C, will take longer the lower the temperature employed in the range 100°C to 175°C. Thus, with a 5 wt.% P₂s₅ or P₂0, treat rate, some 6 hours at 125°C or 2 hours at 150°C could be required. It is preferred to employ short periods, and hence the higher temperatures.

Any hydrolysis, and the further reaction which is conducted (for example neutralisation), may be at any suitable temperature. Thus it may be in the aforesaid 100°C to 175°C range. Preferably, however. the temperature is lower than in the first reaction step, being suitably in the range 120°C to 140°C, preferably about 125°C to 140°C. Again it is found in general that longer periods of time are required for the lower temperatures in the range. Normally one hour is required for a neutralization at 140°C.

It is preferred to employ the oxide, hydroxide or acetate of the desired metal(s) for forming the metal compound(s). Other anions are possible, for example formate, propionate. It is highly preferred to employ as anion one which will give rise to easily removable gaseous or liquid reaction by-products.

Bitumens which can be modified in accordance with the present invention are non- oxidised bitumens or non-blown bitumens, and include natural bitumens or a mineral pitch or a tar obtained as a product from coal or oil. Preferably a petroleum bitumen is employed; such as is obtained as the residue from vacuum distillation of crude oil. If desired, only a portion of such a residue may be employed, for example the precipitated asphalt obtained on treating the residue with a lower alkane, for example propane. The invention is especially suitable for use with penetration grades of bitumen, such as those having (i) a softening point (R Et B) not above 45°C, suitably from 30°C to substantially 40°C, and (ii) a corresponding penetration (units of 0.1 mm at 25°C-ASTM D 5) of from 300 to 80.

The preferred chemically modified bitumens of the invention are those having the metal compound of the phosphorus-containing groups. It is possible to obtain such a modified bitumen having intrinsic elastic properties due to the interaction between the modified molecules of the bitumen and the metal ions introduced into the system during the further reaction, for example neutralization. Such a modified bitumen is very suited for use as a binder giving surfaces prepared therewith (a) improved resistance to fatigue, without adversely affecting the resistance to permanent deformation, and (b) increased ravelling resistance.

By way of illustration of the invention, two samples of a petroleum bitumen, of 41 °C softening point (R & B) and approximately 200 penetration, were taken. Both were heated for 6 hrs. at 150°C with 5 wt.% (calculated as phosphorus and based on the bitumen), one with P₂S₅ the other with P 205. Properties of the P₂0₅-treated bitumen were measured. Substantially complete neutralization of both was thereafter effected employing Ca, Ba and Zn compounds in solid form. Properties of the resultant products were measured. The results are shown in the following Tables 1 and 2.

Relaxation time and initial tensile modulus were measured according to the Tobolski method in Section 9 of "Properties and Structure of Polymers", by A. V Tobolski, published by J. Wiley and Sons, 1960 Edition.

For use in roadmaking a suitable procedure would be to mix the modified bitumen of the invention (very preferably the metal compound type), preheated to 150°C to 170°C, preferably 160°C, with aggregate preheated to a similar temperature. The mixing and laying would be in conventional manner. Thus the benefits of the modified bitumen of the invention can be obtained without recourse to new roadmaking processes and apparatus. Some 6 parts of the modified bitumen per hundred parts of aggregate may be employed. The modified bitumen may itself be first mixed with a filler, suitably up to a 1:1 ratio modified bitumen to filler.

For purposes of comparison, the same petroleum bitumen starting material was treated with phosphoric acid (5 wt.% calculated as phosphorus and based on the bitumen). Reaction was attempted over a period of about 3 hours at 150°C.

The softening point of the product after this treatment had only risen to 43°C, that is to say by only 2°C.

The product was then treated with 6.2 wt.% zinc oxide, but it was found that there were no material differences in the properties of the thus treated product from the phosphoric acid treated material.

Hence there had been no material modification of the starting bitumen on employing phosphoric acid and there were substantially no phosphorus containing functional groups present for reaction with the zinc oxide.

## Claims

1. A chemically modified bitumen possessing phosphorus-containing groups, characterised in that said groups have been reacted with a compound of a metal, preferably a polyvalent metal, or with an ammonium compound or an amine.

2. A chemically modified bitumen as claimed in claim 1, wherein the metal is calcium, barium or zinc.

3. A chemically modified bitumen as claimed in claim 1 or claim 2, wherein said phosphorus-containing groups are phosphonic or thiophosphonic groups.

4. A process for the production of a chemically modified bitumen comprising reacting the bitumen with a phosphorus-containing compound, characterised by further reacting phosphorus-containing groups in the product, directly or after hydrolysis of that product, with a metal compound, an ammonium compound or an amine.

5. A process as claimed in claim 4, wherein the further reaction employs an oxide, hydroxide or acetate of a metal, preferably calcium, barium or zinc.

6. A process as claimed in claim 4 or claim 5, wherein the further reaction is conducted at a temperature in the range 120°C to 140°C.

7. A process as claimed in any one of claims 4 to 6, wherein the phosphorus-containing groups are thiophosphonic or phosphonic groups.

## Patentansprüche

1. Chemisch modifiziertes Bitumen, das Phosphor enthaltende Gruppen besitzt, dadurch gekennzeichnet, daß diese Gruppen mit einer Verbindung eines Metalls, vorzugsweise eines mehrwertigen Metalls oder einer Ammoniumverbindung oder einem Amin umgesetzt worden sind.

2. Chemisch modifiziertes Bitumen nach Anspruch 1, dadurch gekennzeichnet, daß das Metall Calcium, Barium oder Zink ist.

3. Chemisch modifiziertes Bitumen nach Anspruch 1 oder 2, dadurch gekennzeichnet, daß die Phosphor enthaltenden Gruppen Phosphon-oder Thiophosphongruppen sind.

4. Verfahren zur Herstellung eines chemisch modifizierten Bitumen, bei dem das Bitumen mit einer Phosphor enthaltenden Verbindung umgesetzt wird, dadurch gekennzeichnet, daß Phosphor enthaltenden Gruppe in dem Produkt direkt oder nach Hydrolyse des Produkts mit einer Metallverbindung, einer Ammoniumverbindung oder einem Amin weiter umgesetzt werden.

5. Verfahren nach Anspruch 4, dadurch gekennzeichnet, daß in der weiteren Umsetzunc ein Oxid, Hydroxid oder Acetat eines Metalls, vorzugsweise von Calcium, Barium oder Zink verwendet wird.

6. Verfahren nach Anspruch 4 oder 5, dadurch gekennzeichnet, daß die weitere Umsetzung bei einer Temperatur im Bereich von 120 bis 140°C erfolgt.

7. Verfahren nach einem der Ansprüche 4 bis 6, dadurch gekennzeichnet, daß die Phosphor enthaltenden Gruppen Thiophosphonoder Phosphongruppen sind.

## Revendications

1. Bitume chimiquement modifié, possédant des groupes contenant du phosphore, caractérisé en ce qu'on a fait réagir ces groupes sur un dérivé méallique, de préférence d'un métal polyvalent, ou sur un dérivé d'ammonium ou une amine.

2. Bitume chimiquement modifié selon la revendication 1, caractérisé en ce que le métal est le calcium, le baryum ou le zinc.

3. Bitume chimiquement modifié selon l'une quelconque des revendications 1 ou 2, caractérisé en ce que les groupes contenant du phosphore sont des groupes phosphoniques ou thiophosphoniques.

4. Procédé pour la production d'un bitume chimiquement modifié, consistant à faire réagir le bitume sur un composé contenant du phosphore, caractérisé en ce qu'il consiste à faire réagir ensuite les groupes contenant du phosphore du produit, directement ou après hydrolyse de ce produit, sur un composé métallique, un dérivé d'ammonium ou une amine.

5. Procédé selon la revendication 4, caractérisé en ce que la seconde réaction utilise un oxyde, un hydroxyde ou un acétate métallique, de préférence de calcium, de baryum ou de zinc.

6. Procédé selon l'une quelconque des revendications 4 ou 5, caractérisé en ce que la seconde réaction se déroule à une température comprise entre 120 et 140°C.

7. Procédé selon l'une quelconque des revendications 4 à 6, caractérisé en ce que les groupes contenant du phosphore sont des groupes thiophosphoniques ou phosphoniques.
